

S. A. FLOWER.  
FIBROUS LUBRICATING PACKING.  
APPLICATION FILED FEB. 18, 1908.

911,121.

Patented Feb. 2, 1909.



Witnesses  
Martin Zimansky.  
Signed Schuler

Samuel A. Flower <sup>Inventor</sup>  
By his Attorney Ade Bomewill

# UNITED STATES PATENT OFFICE.

SAMUEL A. FLOWER, OF NEW YORK, N. Y.

## FIBROUS LUBRICATING-PACKING.

No. 911,121.

Specification of Letters Patent.

Patented Feb. 2, 1909.

Application filed February 18, 1908. Serial No. 416,634.

*To all whom it may concern:*

Be it known that I, SAMUEL A. FLOWER, a citizen of the United States, and a resident of the borough of Manhattan, in the county 5 of New York and State of New York, have invented certain new and useful Improvements in Fibrous Lubricating-Packings, of which the following is a specification.

This invention relates to a fibrous lubricating packing and process for making the same. Its specific object is to produce a fibrous packing which comprises fire-proofed 10 resilient non-absorbent fibers, and an absorbent fiber or material not subject to self-heating supported in proper operative position by the said resilient fibers.

In the accompanying drawing, which exemplifies the packing, the resilient fibers are shown at 10, with the absorbent material 11. 20 To prepare the packing I mix by weight about fifty parts of cocoa nut fiber and about fifty parts istle hemp, with twelve parts of muriate of ammonia, six parts of sulfate of soda, two parts of sulfate of copper and four 25 parts of borax. The mixture is heated to the boiling point for about twenty minutes after which the fibers are dried. These steps increase the natural resiliency of the fibers, fills the pores thereof to make them non- 30 absorbent and fire-proofs them. I then take by weight 100 parts of jute, or fifty parts of cotton yarn, and fifty parts of jute yarn and submerge them in a solution of one part of bichlorid of mercury, with sixty parts of 35 water for one hour, after which the jute and cotton yarn are dried. This produces an absorbent material not subject to self-heating. Then one part by weight of the prepared fire-proofed resilient fiber is mixed 40 with three parts by weight of the prepared absorbent material to produce the lubricating packing. The product thus obtained is specially applicable as a medium for lubricating car axles. The resilient fibers of the 45 packing easily withstand the shocks consequent to the rough service of a car axle, and

are not subject to destruction by reason of the heating of said axle, and will hold the absorbent material in proper position in a journal box. The capillary attraction of the absorbent material will lubricate the journal of a journal box by conducting a lubricant to the surface of the journal. The efficiency of the resilient fiber is increased by reason of its pores not absorbing any of the lubricant, and the efficiency of the absorbent material is increased by reason of its not being subject to self-heating.

The invention may be modified by using for resilient fiber either wholly the cocoa nut 60 fiber or the istle hemp, and the absorbent material may be either wholly cotton yarn, jute yarn, or jute.

Having described my invention, I claim:

1. A fibrous lubricating packing comprising a resilient fire-proofed fiber and an absorbent material.

2. A fibrous lubricating packing comprising a resilient fire proofed fiber and a non-self-heating absorbent material.

3. A fibrous lubricating packing comprising fire proofed resilient cocoanut fiber and istle hemp, and a non-self-heating absorbent material.

4. A fibrous lubricating packing comprising a resilient fire proofed fiber and non-self-heating cotton yarn.

5. A fibrous lubricating packing comprising fire proofed resilient cocoanut fiber and istle hemp, and non-self-heating absorbent 80 cotton yarn.

6. A fibrous lubricating packing comprising fire proofed resilient istle hemp and non-self-heating cotton yarn.

Signed at the borough of Manhattan in 85 the county of New York and State of New York this 13th day of February A. D. 1908.

SAMUEL A. FLOWER.

Witnesses:

MARTIN ZIMANSKY,  
M. H. COOK.